

Jan. 3, 1950

J. A. BALL ET AL

2,492,954

PHOTOGRAPHIC FOUR-COLOR LIGHT-SENSITIVE  
STRIPPING ELEMENTS  
Filed Dec. 24, 1947



INVENTORS:  
JOSEPH ARTHUR BALL,  
ANDREW BRADSHAW JENNINGS  
and OTIS WILLARD MURRAY

BY

*Lynn Barrett Morris*

ATTORNEY

## UNITED STATES PATENT OFFICE

2,492,954

PHOTOGRAPHIC FOUR-COLOR LIGHT-  
SENSITIVE STRIPPING ELEMENTS

Joseph Arthur Ball, Los Angeles, Calif., Andrew Bradshaw Jennings, New Brunswick, N. J., and Otis Willard Murray, Burbank, Calif., assignors to E. I. du Pont de Nemours & Company, Wilmington, Del., a corporation of Delaware

Application December 24, 1947, Serial No. 793,724

3 Claims. (Cl. 95—2)

1

This invention relates to photography and, more particularly, to a stripping film for four-color photography. Still more particularly it relates to a photographic element provided with four differentially sensitized emulsion layers, three of which can be stripped from the support during processing.

An object of this invention is to provide new photographic elements which are useful in processes of four-color photography. Another object is to provide such elements which can be used to readily obtain four individual color records. A further object is to provide a monopack film element with four differentially sensitized layers from which four color records can be easily separated and processed individually. A still further object is to provide novel processes for obtaining color separation records from such elements. Still other objects will be apparent from the following description of the invention.

The novel photographic elements of this invention consist of a support, such as a transparent film base, provided with a stratum of non-halation material having superposed on one side thereof in order (a) a hydrophilic colloid-silver halide emulsion layer which is sensitive to light in the red region of the spectrum having strong sensitivity in the 605 to 670 millimicron region; (b) a stripping separator layer which preferably contains a small amount of a light filter dye for layer (a); (c) a hydrophilic colloid silver halide emulsion layer which is sensitive to green light possessing its maximum sensitivity between 545 and 575 millimicrons; (d) a stripping layer containing a filter dye to which the next layer (e) is effectively sensitive; (e) a hydrophilic colloid-silver halide emulsion layer which has an extra range of strong sensitivity at 490 to 535 millimicrons; (f) a stripping layer containing a yellow filter dye or pigment; and, finally, (g) a hydrophilic colloid-silver halide emulsion layer which is sensitive to blue and violet light only.

It is to be understood that each of the silver halide emulsion layers are inherently sensitive to blue light, in addition to having the extra sensitivity specified above. However, the light filter layers prevent the lower layers from being exposed in the blue region of the spectrum.

The novel photographic elements of this in-

vention are especially useful in the processes of four-color photography disclosed in Ball application Serial Number 771,790, filed September 2, 1947. The photographic elements can be used to form four individual color separation records from which four color separation positive silver image records can be printed as provided in said application. The latter image records can then be converted into colored images having the absorption peaks and characteristics taught in said application. The colored images may then be superposed in register to reproduce a multicolor picture.

The stripping layers of the elements may be composed of various materials which are softened or dissolved by water. Thus, they may be composed of any water-soluble colloid (viz. which has a marked solubility in water at 20° C.) of natural or synthetic type. Suitable colloids include water-soluble cellulose derivatives, e. g., low substituted cellulose ethers, such as methyl cellulose, ethyl cellulose, and benzyl cellulose, cellulose esters having solubilizing acid salt groups, e. g., sodium, potassium, and ammonium salts of cellulose acid phthalate, cellulose ether acids, e. g., sodium cellulose glycolate, casein gelatin mixtures, water-soluble synthetic resins, e. g., polyvinyl alcohol and esters.

In the preferred aspect of the invention, the stripping layers are composed of a water-soluble but photographic alkaline developer insoluble colloid. Preferred colloids of this type are composed of water-soluble macromolecular acetals of vinyl alcohol polymers with an aldehyde containing sulfonic acid and/or carboxylic acid groups or their water-soluble salts, e. g., alkali metal, ammonium or amine salts.

The water-soluble macromolecular acetals can be made by the reaction of a vinyl alcohol polymer, including interpolymers, with an aldehyde containing a sulfonic acid or a carboxylic acid group under acetal-forming conditions. For example, the acetalization may be conveniently carried out in solution or suspension in water or an organic solvent or diluent using a catalyst such as phosphoric acid, sulfuric acid, hydrochloric acid, etc. Suitable procedures and aldehydes are described in United States Patent 2,310,943 and in German Patent No. 643,650. The free acid groups can be converted into salt groups

by a simple neutralization as described above and in the United States patent.

Partially and completely hydrolyzed polyvinyl alcohols of low, intermediate, and high viscosity, having a molecular weight of 5,000 to 50,000 and hydrolyzed interpolymers of vinyl esters with one or less equivalent of a terminally unsaturated interpolymerizable organic compound can be used in preparing the vinyl alcohol acetals of aldehydes containing carboxylic or sulfonic acid groups. In general, such polymers having for each 100 carbon atoms between 20 and 50 free non-phenolic hydroxyl groups are useful.

Preferred water-soluble, macromolecular, neutralized acetals of vinyl alcohol polymers used in accordance with this invention are prepared by acetalization from (1) polyvinyl alcohol of high molecular weight (viscosity of 4% aqueous solution at 20° C., 40 to 60 centipoises), (2) polyvinyl alcohol of medium molecular weight (viscosity of 4% aqueous solutions at 20° C., 15 to 30 centipoises) substituted on 40 to 60% of the hydroxyl groups with acetate, propionate, acetal, propional, and butyral groups, (3) 75 to 100% hydrolyzed interpolymers of vinyl acetate with 0.05 to 0.5 mol equivalents of terminally unsaturated monolefins, e. g., ethylene, such as described in Roland United States Patent No. 2,386,347, and (4) completely hydrolyzed interpolymers of vinyl acetate with minor portion (less than 50%) of polymerizable vinyl or vinylidene compounds, for example, vinyl chloride, vinyl cyanide, alkyl methacrylates, e. g., methyl and ethyl methacrylate, etc., with an aldehyde containing carboxylic or a sulfonic acid group.

The preferred polyvinyl acetals have the above properties and, in addition, are colorless or substantially colorless and are free from color former nuclei.

The degree of substitution of the acetal groups may vary over a wide range. Thus, vinyl alcohol polymers having between 5 and 60% of the hydroxyl groups acetalized with acidic aldehydes have been found useful. However, it has been found that the best results are obtained when between 10 and 35% of the hydroxyl groups are acetalized with the acidic aldehydes. The total acetal content based on these figures will vary depending on the hydroxyl content of the polymer, but it has been found that the best results are obtained when between 5 and 17% of the carbon atoms of the polymer chain contain the acetal groups with  $-\text{COO}-$  and  $-\text{SO}_3-$  radicals. The acetals having this degree of substitution, however, may be used in the form of the free acids but are preferably used in the form of the water-soluble salts which are soluble to the extent of at least 5% at temperatures below 30° C. in methanol or ethanol containing up to 20% of water.

While any aldehyde containing a free carboxylic or sulfonic acid radical may be used in preparing these acetals, those having a molecular weight of less than 200 are preferred as, in general, they react more readily and completely. These aldehyde-acids may be aromatic, aliphatic, or mixed aromatic-aliphatic.

The colloid stripping materials, e. g., the water-soluble macromolecular acetals of vinyl alcohol polymers described above can be applied to the contiguous layer from a solution or dispersion in the same general manner that gelatin overcoatings are applied. The acetal layers so applied should be of such a thickness that they may be readily stripped from the layer on which they

are coated. The exact thicknesses can be readily determined by experiment. Thicknesses of 0.0001 to 0.0005 inch, in general, are satisfactory. Materially thinner layers, e. g. 0.05 to 2.0 microns, in general, adhere quite firmly. They may be applied from aqueous or organic solvent solutions. Useful solvents are the water-soluble alcohols, e. g., methanol, ethanol, acetone, dioxane, etc. Mixtures of such solvents with water are quite useful. The coating solutions are preferably substantially neutral. Their pH can be adjusted by neutralizing the free acid groups with bases capable of yielding water-soluble salts, e. g. alkali metals, ammonia, and amines. Various filter dyes or pigments are added to the coating solutions prior to depositing the layers on the silver halide emulsion layers.

In using the novel film elements, the emulsion surface is placed nearest to the lens in the camera and it is then exposed to a multicolor object field. The exposed film is then developed in an alkaline photographic developing bath whereby four color-separation negative silver image records are formed in the respective layers of the monopack element. It is then treated in an acid stop bath. The film element is then immersed in a water bath whereby the bond between the image bearing layers and the water-soluble colloid weakens or dissolves. The image bearing layers are successively removed and can be individually treated. They may, for example, be fixed, washed, and dried resulting in four developed color separation negatives suitable for registration printing on separate film elements to produce positives on which exposed film elements can be color developed in the appropriate bath to form a dye image of the proper color in situ with a silver image as described in aforesaid Ball application. The silver and silver salts are removed leaving a dye image. The four dye image positive records are superposed in register which results in a multicolor positive picture.

The invention will be further illustrated by the following example.

#### Example

A cellulose acetate film base is coated on its rear surface with an antihalation layer composed of o-sulfobenzaldehyde acetal of polyvinyl alcohol and finely divided or comminute silver. The front surface is then provided in order with the following seven layers and having the construction set forth in Fig. 1 of the accompanying drawing which forms part of this specification. Layer 1 is a gelatino-silver iodobromide emulsion layer having a coating weight of 50 milligrams of silver bromide per square decimeter and containing 1,1'-diethyl-2,2'-carbocyanine iodide which confers sensitivity to about 670 millimicrons.

Layer 2 is composed of a water-soluble, developer insoluble o-sulfobenzaldehyde acetal of polyvinyl alcohol uniformly dyed with Congo Red (Colour Index No. 370).

The "Color Index" herein referred to is that by F. M. Rowe, published by The Society of Dyers and Colorists, England, first ed., January, 1924.

Layer 3 is a gelatino-silver iodobromide emulsion having a coating weight like layer 1 and containing Erythrosine which confers a sensitivity having a maximum at 570 millimicrons.

Layer 4 is similar to layer 2 but contains Wool Orange A (Colour Index No. 151) in place of Congo Red.

Layer 5 is a gelatino-silver iodobromide emulsion having a coating weight like layer 1 and con-

taining 3,3'-diethyl-9-methyl oxy carbocyanine iodide and has a maximum sensitivity at 514 to 520 millimicrons.

Layer 6 is similar to layer 2 but contains Tartrazine-O (Colour Index No. 640) in place of Congo Red.

Layer 7 is a blue-sensitive gelatino-silver iodobromide emulsion having a coating weight of 50 milligrams of silver bromide per square decimeter.

The film is exposed in a camera to a natural multicolor scene and is then developed for seven minutes in a solution of the following composition:

|                               |        |      |
|-------------------------------|--------|------|
| Hydroquinone                  | grams  | 7.5  |
| p-N-methylaminophenol sulfate | do     | 5.0  |
| Sodium sulfite (anhydrous)    | do     | 60.0 |
| Sodium carbonate (anhydrous)  | do     | 50.0 |
| Potassium bromide             | do     | 15.0 |
| Water to                      | liters | 1.0  |

The developed film is then treated for one minute in a stop bath of the composition:

|                   |        |      |
|-------------------|--------|------|
| Acetic acid (28%) | Volume | 1.0  |
| Water             |        | 20.0 |

The outer layer 7 is then pressed into intimate contact with a second registered support comprising a transparent film base coated with a gelatin layer having a coating weight of about 75 milligrams of silver bromide per square decimeter which had been wetted with water to promote adhesion between the gelatin surfaces. The water weakens the bond of layer 6 whereby layer 7 is stripped from the element.

It is possible to alter the time of immersion in the stop bath and the state of water absorption of the gel blank so that the outermost image layer may be removed without weakening the adhesion of the under layers.

Layers 5 and 3 are transferred to separate film elements bearing gelatin layers in like manner. By reimmersion in the stop bath and bringing into contact with other wetted blanks, the remaining layers may be successively transferred, in each case regulating the time of immersion and water content of the blank so as to remove only the desired layer. The resulting four separate color separation records are fixed, washed, and dried and used to print onto positive film elements which can be color developed, fixed, washed, and dried as described in the aforescribed Ball application.

A similar element can be made by substituting for the yellow filter material of layer 6 other dyes or pigments including Auramine O (Color Index No. 655), Quinoline Yellow (Color Index No. 801), Naphthol Yellow S (Color Index No. 10), and yellow colloidal silver.

Inert salts, e. g., sodium sulfate (about 120 grams per liter) can be added to the stop baths to prevent excessive softening of the stripping layer if desired.

Similarly in place of the sensitizing dyes for layer 1, there may be substituted 3,3'-diethyl selenacarbocyanine iodide or 2(p-dimethylamino-styryl-6-ethoxybenzothiazole ethyl bromide. Additional sensitizing dyes suitable for layer 3 include 3-ethyl-5(3-ethyl-2(3)-benzoxazolylidene)-ethylidene-rhodanine and 1,1'-diethyl pseudocyanine-p-toluene sulfonate. In place of the sensitizers for layer 5, there can be used 3,3'-

diethyl-oxy carbocyanine iodide or 3,3'-diethyl-5,5'-di-methyl oxy carbocyanine iodide.

In place of the filter dyes for layer 4, there can be used Pontacyl Brilliant Orange 2R, Colour Index #2176, and Lake Scarlet R, Colour Index #79.

Various other stripping layers can be used in place of the specific acetal of the example. They may be composed of any of the materials described above for this purpose. Additional suitable coating compositions for this purpose include the following:

*Solution A*

|                                       |       |       |
|---------------------------------------|-------|-------|
| Casein                                | grams | 20.0  |
| Water                                 | cc    | 100.0 |
| Na <sub>2</sub> CO <sub>3</sub> (20%) | cc    | 6.8   |
| Gelatin                               | grams | 1.0   |
| Mannitan monolaurate (10%)            | cc    | 5.0   |
| Water                                 | cc    | 50.0  |

*Solution B*

|                              |       |       |
|------------------------------|-------|-------|
| Corn dextrine                | grams | 10.0  |
| Water                        | cc    | 100.0 |
| Ethanol                      | cc    | 20.0  |
| Saponin solution             | cc    | 10.0  |
| Sodium dodecyl sulfate (10%) | cc    | 2.0   |

*Solution C*

|                                  |       |       |
|----------------------------------|-------|-------|
| Cellulose acetate-acid phthalate | grams | 5.0   |
| Na <sub>2</sub> CO <sub>3</sub>  | cc    | 10.0  |
| Water                            | cc    | 150.0 |
| Ethanol                          | cc    | 50.0  |
| Gelatin                          | grams | 5.0   |
| Water                            | cc    | 100.0 |

*Solution D*

|                                        |       |        |
|----------------------------------------|-------|--------|
| Cellulose acetate (17% acetyl content) | grams | 10.0   |
| Water                                  | cc    | 1000.0 |

It is to be understood, however, that the light-screening or filter dyes or pigments are to be added to said solutions before coating.

The silver halide emulsion layers are preferably composed of gelatin as the binding agent. However, various other natural or synthetic hydrophilic colloids can be used, if desired, e. g., agar agar, albumen, nylon, polyvinyl acetals, the hydrolyzed ethylene/vinyl acetate interpolymers of Patent No. 2,397,866, etc.

An advantage of the invention resides in the fact that it provides a novel and practical unitary element for four-color photography. A further object is that the element can be made in a simple and economical manner. A further advantage is that it is unitary and offers no difficulty in fitting it to cameras. It can be readily processed to yield four-color separation records which can be separately handled.

What is claimed is:

1. A multilayer photographic element comprising a transparent film base having superposed thereon in order a hydrophilic colloid silver halide emulsion layer which has an extra band of sensitivity in the red region of the spectrum with a maximum sensitivity at a position within the

range from 605 to 670 millimicrons, a stripping separator layer composed of a developer-insoluble, water-soluble colloid containing a light-filter dye for the aforesaid first layer, a hydrophilic colloid silver halide emulsion layer which has an extra band of sensitivity in the yellow region of the spectrum with a maximum sensitivity at a position within the range 545 to 575 millimicrons, a stripping layer composed of a developer-insoluble, water-soluble colloid containing a filter dye which absorbs light to which the next-men-

7  
tioned layer is effectively sensitive, a hydrophilic colloid silver halide emulsion which has an extra band of sensitivity in the green region of the spectrum with a maximum sensitivity at a position between 490 and 535 millimicrons, a stripping layer composed of a developer-insoluble, water-soluble colloid containing a yellow filter material and finally a hydrophilic colloid silver halide emulsion layer which is sensitive to blue light only.

2. An element as set forth in claim 1 wherein the hydrophilic colloid is gelatin.

3. An element as set forth in claim 1 wherein said silver halide emulsion layers contain gelatin as the binding agent and the stripping layers are 15 composed of a water-soluble acetal of a vinyl alcohol polymer with an aldehyde containing a

8  
group taken from the class consisting of free carboxylic acid groups, free sulfonic acid groups, and their water-soluble salts.

JOSEPH ARTHUR BALL.  
ANDREW BRADSHAW JENNINGS.  
OTIS WILLARD MURRAY.

REFERENCES CITED

10 The following references are of record in the file of this patent:

UNITED STATES PATENTS

| Number    | Name        | Date          |
|-----------|-------------|---------------|
| 2,167,732 | Verkinderen | Aug. 1, 1939  |
| 2,182,814 | Marasco     | Dec. 12, 1939 |
| 2,415,442 | Rackett     | Feb. 11, 1947 |